

[54] FLAME-RETARDANT TEXTILES BY  
REACTION OF CELLULOSE WITH THE  
ADDUCT OF PHOSPHORUS TRICHLORIDE  
AND N,N-DIMETHYLFORMAMIDE

[75] Inventors: Tyrone L. Vigo, Kenner; Clark M. Welch, Metairie, both of La.; Anna M. Collins, College Park, Ga.

[73] Assignee: The United States of America as  
represented by the Secretary of  
Agriculture, Washington, D.C.

[22] Filed: Jan. 28, 1974

[21] Appl. No.: 437,096

[52] U.S. Cl. .... 8/188; 8/116 P; 260/219

[51] Int. Cl.<sup>2</sup> .... D06M 13/46

[58] Field of Search .... 8/116 P, 188

## [56] References Cited

### UNITED STATES PATENTS

2,489,225 11/1949 Morris ..... 260/230

### OTHER PUBLICATIONS

Vigo et al., "—Reaction of Cellulose with PCl<sub>3</sub>—DMF Adduct," Journal of Applied Polymer Science, Vol. 17, No. 2, pp. 571-584 (1973), regis-

tered publication date of Mar. 13, 1973.

Primary Examiner—Murray Tillman

Assistant Examiner—Arthur H. Koeckert

Attorney, Agent, or Firm—M. Howard Silverstein; Max D. Hensley

## [57] ABSTRACT

The preparation in textile form of a cellulose N,N-dimethylorthoformamoylphosphorochloridite ester possessing flame and wrinkle resistance is described. The preparation is accomplished by preswelling the cellulose for 1 to 60 minutes in N,N-dimethylformamide, followed by reaction of the cellulose with 1-30% concentrations of phosphorus trichloride-N,N-dimethylformamide adduct in excess N,N-dimethylformamide as solvent, with or without an inert diluent, at 20-60°C for 1 to 180 minutes. After the reaction has been carried out to the desired extent of completion the modified cellulose is washed with an inert solvent. The modified cellulose contains nitrogen, phosphorus, and chlorine in a ratio of 1:1:1. If desired, the product can be freed of chlorine by subsequent washing in ice water, or may be used directly as an intermediate for further modification.

8 Claims, No Drawings

**FLAME-RETARDANT TEXTILES BY REACTION  
OF CELLULOSE WITH THE ADDUCT OF  
PHOSPHORUS TRICHLORIDE AND  
N,N-DIMETHYLFORMAMIDE**

This invention relates to a method of imparting flame and wrinkle resistance to cellulosic textile materials by reaction of the cellulose with an adduct which phosphorus trichloride forms with N,N-dimethylformamide. More specifically, the present invention relates to the conversion of fibrous cellulose in the form of yarn or fabric into phosphorus-, nitrogen-, and halogen-containing cellulosic textiles having flame resistance and improved wrinkle recovery, by reaction of the cellulose with phosphorus trichloride-N,N-dimethylformamide adduct in aprotic solvents.

The main object of the present invention is to impart flame resistance to cellulosic textiles by chemical modification of the cellulose by means of a phosphorus trichloride adduct with N,N-dimethylformamide.

A second object of the present invention is to provide a means of introducing a limited degree of cellulose crosslinking in cellulosic fabrics, so as to impart increased wrinkle resistance in the wet and dry states.

A third object of the present invention is to provide a means of introducing phosphorus- and nitrogen-containing substituents, as well as chlorine, into fibrous cellulose while retaining the fiber structure, whiteness, and most of the tensile strength of the original untreated cellulose.

Although the prior literature contains studies on the reaction of phosphorus trichloride with chemically substituted cellulose, no method has been previously proposed for the treatment of unsubstituted fibrous cellulose with this reagent with retention of the original fiber structure of the cellulose. The nature of the products formed in prior processes are different from those in our process, inasmuch as the prior processes introduce ether, ester, or olefinic substituents into the cellulose prior to its reaction with phosphorus trichloride. Some of the prior processes depend for their effectiveness on bringing the cellulose derivative into solution so as to facilitate reaction with phosphorus trichloride.

For example, in U.S. Pat. No. 2,489,225 (Nov. 22, 1949), phosphorus trichloride is reacted with soluble cellulose ether or ester derivatives. The degree of substitution of the modified cellulose ether or ester is that necessary to render the cellulosic material soluble in organic solvents or in phosphorus trichloride. Such a process is not suitable for treatment of native cellulose when it is desired to retain the fiber, yarn or fabric structure which the cellulose originally possesses. Likewise, recent work by Dimitrov, et al. (Cellulose Chem. Technol. 1968, 2(4), 375-389) describes the reaction of phosphorus trichloride with a cellulosic derivative (5,6-celluloseen) in which an olefinic group must be present in order for the cellulose to react with the phosphorus trichloride. The phosphorus halide adds across the olefinic double bond in this instance.

The present invention makes it possible for the first time to react phosphorus trichloride with unsubstituted cotton cellulose under mild reaction conditions without the need of having  $\text{PCl}_3$ -reactive substituents on the cellulose. This is accomplished by the reaction of a N,N-dimethylformamide adduct of phosphorus trichloride with the cellulose. Such a reaction system controls the reactivity of the phosphorus trichloride, avoids degradation and tendering of the cellulose, precludes the necessity of having other substituents on the cellulose to obtain reaction with phosphorus trichloride, and permits retention of the original fiber, yarn and fabric structure by the cellulosic textile.

Another major advantage of the present process over prior art is that it simultaneously introduces, in a one-step process, nitrogen as well as phosphorus into the cellulose, and in doing so, produces a product having high flame resistance as well as improved wrinkle recovery. It is well known that nitrogen and phosphorus have a synergistic effect in imparting flame retardancy to cellulose.

A further advantage of the present process is that pretreatment of the cellulose with N,N-dimethylformamide activates the cellulose, and greatly increases its rate of reaction towards the phosphorus trichloride-N,N-dimethylformamide adduct. Such an increase is essential to obtain the high phosphorus and nitrogen contents necessary in the cellulosic product for adequate flame and wrinkle resistance. Other advantages will become apparent in the description that follows.

The processes of this invention are applicable to cellulose derived from cotton or wood pulp, which cellulose may be native, mercerized, or regenerated, and which may be in the form of loose fibers, silver, yarn or fabric.

The above advantages of the present invention are unexpectedly obtained by using a phosphorus trichloride adduct with N,N-dimethylformamide in the treatment of cellulose.

The phosphorus trichloride adduct with N,N-dimethylformamide is formed by reaction of phosphorus trichloride with N,N-dimethylformamide at 0°-30°C in the absence of air and moisture. The reaction is nearly instantaneous, and may be carried out using excess N,N-dimethylformamide as both reactant and solvent, or may be carried out as described in the literature [T. D. Smith, J. Chem. Soc., 841 (1966)] using an inert diluent such as carbon tetrachloride. The mole ratio of phosphorus trichloride to N,N-dimethylformamide in the adduct is known to be 1:2. The structure of the adduct has previously been established by Smith as  $\text{Cl}-\text{P}-(\text{OCH}=\text{N}(\text{CH}_3)_2)_2^{++} 2\text{Cl}^-$ .

In carrying out the processes of the present invention, the 1:2 adduct of phosphorus trichloride with dimethylformamide does not need to be isolated or purified, but can be used directly as formed in solution in excess dimethylformamide, with or without other diluents present. The presence of excess dimethylformamide minimizes cellulose degradation and tendering during reaction of the adduct with the cellulose, and is therefore preferred. The reaction between cellulose and the adduct is thought to proceed as follows:





where Cell-OH is a portion of a molecular chain of cellulose and R is a methyl group. The product, herein referred to as a cellulose N,N-dimethylorthoformamoylphosphorochloridite ester, is found to contain phosphorus, nitrogen, and chlorine in an atomic ratio of 1:1:1. Subsequent treatment with water produces the following reactions:



The relative proportions of nitrogen and chlorine lost depends on the relative extent to which these hydrolytic reactions are carried to completion. Formation of a labile formate derivative during hydrolysis is indicated by increased infrared absorption at 5.75-5.85  $\mu$  characteristic of the carbonyl group in formates.

The treatment of cellulose by the processes of the present invention comprises the following steps:

a. immersion of air-equilibrated, fibrous cellulose in textile form in N,N-dimethylformamide at a temperature of about from 20°C to 30°C for a period of from 1 minute to 60 minutes to swell the fibers,

b. removal of excess N,N-dimethylformamide from the swollen cellulose.

c. immersion of the cellulosic textile in a solution containing about from 1% to 30% by weight of the 1:2 adduct of phosphorus trichloride with N,N-dimethylformamide together with an inert aprotic diluent selected from the class consisting of chloroform, carbon tetrachloride, methylene chloride and perchloroethylene at a temperature of from 20°C to 60°C for about from 1 minute to 180 minutes, in order to obtain reaction of the cellulose with the adduct,

d. washing the cellulosic textile with N,N-dimethylformamide to remove unreacted adduct,

e. washing the cellulosic textile with an inert solvent selected from the group consisting of benzene and chloroform, to remove N,N-dimethylformamide,

f. washing the cellulosic textile with ice water, and then washing at room temperature with water containing 0-10% acetic acid, to remove traces of combined chlorine and reagent and solvents, and

g. drying the textile.

The immersion of the cellulose in N,N-dimethylformamide, as specified in step (a) above, is critical to the process, in that this step swells the cellulose fibers and greatly increases the rate of subsequent reaction of the cellulose with the adduct of phosphorus trichloride and N,N-dimethylformamide. The cellulose to be used in this process should be at equilibrium with the atmosphere at ordinary humidity so that the moisture content causes the fibers to be much more accessible to swelling by N,N-dimethylformamide and to subsequent reaction with the adduct of phosphorus trichloride and N,N-dimethylformamide. The cellulose should not be subjected to any deswelling treatment such as oven-

drying, prior to immersion in the N,N-dimethylformamide.

Removal of excess N,N-dimethylformamide or other tertiary amides in step (b) above, may be accomplished by ordinary mechanical methods of wringing, such as passing the fabric through squeeze rolls, centrifugation, draining, or by pressing the cellulose against a filter.

The reaction of the cellulosic textile with the adduct of phosphorus trichloride and N,N-dimethylformamide as specified in step (c) above, in preferably carried out in N,N-dimethylformamide as the reaction solvent, since this solvent maintains the cellulose in a swollen state; and since the above adduct has considerably solubility in this medium. At concentrations above 15% by weight of N,N-dimethylformamide-phosphorus trichloride adduct, it is necessary to use an inert diluent such as chloroform, methylene chloride, carbon tetrachloride, or perchloroethylene, as part of the solvent system to insure solubility of the adduct before it is reacted with the cellulose.

The weight ratio of the phosphorus trichloride-amide adduct to cellulose which may be used can be varied over a wide range. The most practical ratio to use depends to some extent on whether the cellulose is in the form of loose fibers, silver, yarn or fabric, since the reactivity of the cellulose varies with the form of cellulose being treated. The preferred ratio also varies with the degree of flame resistance and improvement in wrinkle recovery desired in the cellulose, but usually is in excess of 1 part by weight of the adduct to 5 parts by weight of the cellulose. The concentration of the phosphorus trichloride-amide adduct may be varied considerably, but above a concentration of 30% by weight, the reactions with cellulose slows down considerably, and little practical benefit results from the use of higher ratios.

By adjusting the phosphorus trichloride-amide adduct concentration and the reaction time, the extent of reaction of the adduct with the cellulose can be varied considerably, so that the phosphorus content obtained in the modified cellulose is in the range of 0.6% to 6%, the nitrogen content is in the range of 0.1% to 2.5%, and the chlorine content is in the range of 0.1% to 6%.

Step (d) removes the unreacted phosphorus trichloride-amide adduct. Step (e) removes N,N-dimethylformamide. Step (e) can be omitted when the modified cellulose is to be water-washed as in step (f). Washing step (f) is omitted when it is desired to maintain the P-Cl bond in the modified cellulose for further reaction with other substrates. The cellulose N,N-dimethylorthoformamoylphosphorochloridite ester obtained can be reacted with active hydrogen compounds such as amines, alcohols, and mercaptans to yield other

derivatives of cellulose in textile form:

During the wash with ice water, partial hydrolysis occurs as already indicated in the above equations, and most of the combined chlorine in the product is removed. A portion of the combined nitrogen in the product is also lost in this washing step. The wash with ice water is preferably followed by a wash with 1-10% aqueous acetic acid when the adduct concentration used in treating the cellulose is 10% or less. The acetic acid decreases the binding of metal ions present in the wash water by the substituted cellulose, and thus renders the flame retardancy more durable to washing.

In the examples that follow, fabric breaking strength (strip method) was determined by the procedure of ASTM-D1682-64, using a Scott tester. Wrinkle recovery was determined by the Monsanto method (ASTM D-1295-67). Flame resistance was measured by the standard vertical flame test described in U.S. Federal Supply Service, "Textile Test Methods," Federal Test Method Std. No. 191, Method 5903.1, and by the match or clock test described by Reeves, et al. [Text. Res. J. 23, 527-532 (1953)]. Durability to laundering of the treated fabrics was determined by repeated washing and drying in an agitator-type washer and a tumble dryer under normal conditions for cotton (10 minutes hot water wash, 30 minutes high temperature drying) using a commercial phosphate detergent. All parts and percentages are by weight. The phosphorus trichloride-amide adduct concentrations specified are based on the 1:2 adduct of phosphorus trichloride with the amide, and in the cases where N,N-dimethylformamide is the amide used, the adduct concentration specified is 2.07 times the percentage by weight of phosphorus trichloride added in making up the treating solution. The cotton cloth used for fabric treatments was desized, scoured, and bleached sateen weighing 8 oz. per sq. yd. N,N-dimethylformamide is hereafter abbreviated DMF.

#### EXAMPLE 1

##### Reaction of Cotton Fabric with Phosphorus Trichloride-DMF Adduct in DMF at Low Adduct Concentrations

Desized, scoured, and bleached 8 oz./yd.<sup>2</sup> cotton sateen fabric was immersed in excess N,N-dimethylformamide (DMF) for 30 minutes at 25°C, put through laboratory wringers to remove excess DMF, and then reacted for 15 minutes at 25°C with 5% phosphorus trichloride-DMF adduct in DMF in a stoppered flask with agitation, utilizing 40 grams of solution per gram of cotton. This solution was prepared by adding 2.4 parts of phosphorus trichloride to 97.6 parts by weight of DMF. The fabric was subsequently washed three times with excess DMF, then with ice water, immersed in 5% aqueous acetic acid for 10 minutes, washed with tap water for 1 minute, and allowed to air-dry to constant weight. The resultant fabric had an add-on of 9.8%, and the following elemental composition: %P, 1.8; %N, 0.6; %Cl, 0.02; %Ca, 0.02. The fabric had a char length of 3.75 inches as measured by the standard vertical flame test and possessed no afterglow; untreated sateen fabric had extensive afterglow, very little char, and burned the entire fabric length (10 inches) under comparable test conditions. The breaking strength of the treated fabric was 90 lbs. while that of the untreated fabric was 137 lbs. The conditioned and wet wrinkle recoveries (warp + fill) of the treated fabric were respectively

215° and 222°, while those of the untreated fabric were respectively 183° and 168°. Fibers of the treated fabric were insoluble in 0.5 M aqueous cupriethylenediamine solution, even after 10 minutes standing, whereas fibers of untreated fabric dissolved within 15-30 seconds. This shows that the treated cotton cellulose was highly crosslinked. The cellulose crosslinking imparted by the process of this invention was responsible for the wrinkle resistance imparted.

#### EXAMPLE 2

##### Reaction of Cotton Fabric with Phosphorus Trichloride-DMF in DMF at Intermediate Adduct Concentrations

Cotton sateen fabric was immersed in excess DMF for 30 minutes at 25°C, put through laboratory wringers to remove excess DMF, then reacted for 15 minutes at 25°C with 15% phosphorus trichloride-DMF adduct in DMF in a stoppered flask with agitation, utilizing 40 grams of solution per gram of cotton. This solution was prepared by adding 7.2 parts of phosphorus trichloride to 92.8 parts of DMF. The fabric was then washed three times with excess DMF, once with chloroform, and allowed to air-dry to constant weight. The resultant fabric had an add-on of 19.0%, a match test angle of 180°, and the following elemental composition: %P, 2.8; %N, 1.1; %Cl, 2.5; %Ca, 0.01, and was suitable for further reaction utilizing the reactive P-Cl linkage. The atomic ratio of phosphorus, nitrogen, and chlorine in this product was 1.3:1.1:1.0, or approximately 1:1:1.

#### EXAMPLE 3

##### Reaction of Cotton Fabric with Phosphorus Trichloride-DMF in DMF-CHCl<sub>3</sub> at High Adduct Concentrations

Cotton sateen fabric was immersed in excess DMF for 30 minutes at 25°C, put through laboratory wringers to remove excess DMF, then reacted for 1 hour at 25°C with 25% phosphorus trichloride-DMF adduct-59% DMF-16% chloroform in a stoppered flask with agitation, utilizing 40 grams of solution per gram of cotton. This solution was prepared by adding 12.1 parts of phosphorus trichloride to 87.9 parts of a 3.7:1 mixture by weight of DMF and chloroform. The fabric was then washed with excess DMF, ice water, and tap water in excess for 30 minutes, and allowed to air-dry overnight. The resultant fabric possessed 3.9% P, 0.6% N, 0.3% Ca, and 0.4% Cl, and had a char length of 2.5 inches. Fibers of the treated fabrics were insoluble in 0.5 M cupriethylenediamine solution indicating the cellulose was highly crosslinked. After 20 standard home launderings (wash and tumble dry cycles) using a commercial phosphate detergent in the wash cycle, the fabric possessed 5.2% P, 0.3% N, 1.2% Ca, and 0.8% Cl, and still passed the standard vertical flame test with a char length of 3.5 inches.

#### EXAMPLE 4

##### Reaction of Cotton Fabric with Phosphorus Trichloride-DMF Adduct in DMF with Omission of Preswelling Step.

Cotton sateen fabric was immersed in 5% phosphorus trichloride-DMF in DMF for 15 minutes at 25°C with agitation, utilizing 40 grams of solution per gram of cotton. This solution was prepared by adding 2.4 parts of phosphorus trichloride to 97.6 parts of DMF. The fab-

ric was then washed with DMF, ice water, 5% aqueous acetic acid for 10 minutes, tap water for 1 minute, and allowed to air-dry. The resultant fabric had a weight gain of only 0.7%, and only 0.1% P, 0.05% N, with trace amounts of chlorine and calcium. Although the fabric possessed no afterglow, it had a 0° angle by the match test, and was therefore unsuitable for testing by the standard vertical flame test method. The results show that it is necessary to preswell the cellulose in DMF to obtain a useful degree of reaction by the processes of the present invention.

## EXAMPLE 5

## Reaction of Cotton Fabric with the Phosphorus Trichloride Adduct of N,N-dimethylacetamide in DMF

Cotton sateen fabric was immersed for 30 minutes in excess DMF, then put through wringers to remove excess DMF, then reacted with agitation in a stoppered flask containing 5% phosphorus trichloride-N,N-dimethylacetamide adduct dissolved in DMF, there being 40 grams of solution per gram of cotton. This reaction was run at 25°C for 1 hr. The solution was prepared by adding 2.2 parts of phosphorus trichloride to 2.8 parts of N,N-dimethylacetamide with cooling to maintain a temperature not exceeding 50°C. The resulting solution was dissolved in 95 parts of DMF. The resultant fabric was washed with DMF, ice water, tap water for 30 minutes, and allowed to air-dry. The fabric, although having no afterglow when ignited, had a match test angle of 0°, and was therefore not acceptable for further flammability testing. Elemental analysis of the fabric gave the following results: % P—0.1, %N—0.15, % Cl—0.03, % Ca—0.13. Conducting the reaction using N,N-dimethylacetamide as the preswelling agent, and dissolving the adduct in N,N-dimethylacetamide gave comparable results. This example proves that N,N-dimethylacetamide cannot be used in place of DMF in the processes of the present invention.

## EXAMPLE 6

## Reaction of Cotton Fabric with Phosphorus Trichloride-N-Methylpyrrolidone Adduct in DMF

Cotton sateen fabric was immersed for 30 minutes in excess DMF, and was then put through wringers to remove excess DMF. The fabric was immersed with agitation in a stoppered flask containing 5.9% phosphorus trichloride-N-methylpyrrolidone adduct dissolved in DMF, there being 40 grams of solution per gram of cotton. The reaction was run at 25°C for 1 hr. The solution was prepared by adding 3.5 parts N-methylpyrrolidone to 2.4 parts of phosphorus trichloride with cooling, and later adding 94.1 parts of DMF. The resultant fabric was washed as in Example 1, and possessed only 0.1% phosphorus, and trace amounts of nitrogen, chlorine, and calcium. It had a match test angle of 0° and was therefore unacceptable for use as a flame-retardant fabric. Repeating the reaction using N-methylpyrrolidone in the preswelling step as well as in the reaction gave comparable results. This example shows that N-methylpyrrolidone cannot be used in place of DMF in the processes of the present invention.

## EXAMPLE 7

## Reaction of Cotton Fabric with Phosphorus Tribromide-N,N-Dimethylformamide Adduct in DMF

Cotton sateen fabric was immersed for 30 minutes in excess DMF, then put through wringers to remove excess DMF, and reacted with agitation in a stoppered flask containing 5% phosphorus tribromide-N,N-dimethylformamide adduct dissolved in DMF utilizing 40 grams of solution per gram of cotton. This solution was prepared by adding 3.2 parts of phosphorus tribromide to 96.8 parts of DMF. The reaction was run for 1 hr. at 25°C. The resultant fabric was washed as in Example 1, and possessed 0.5% P, 0.2% N, 0.1% Br, and trace amounts of calcium. It had a match test angle of 45°, and therefore possessed some flame resistance, but not enough to be of practical benefit. The results show that phosphorus tribromide cannot be substituted for phosphorus trichloride in the processes of our invention.

## EXAMPLE 8

## Reaction of Cotton Yarn with Phosphorus Trichloride-N,N-Dimethylformamide Adduct in DMF

Kiered 12/3 cotton yarn was immersed for 30 minutes in excess DMF, then centrifuged to remove excess DMF, and reacted with agitation in a stoppered flask containing 15% phosphorus trichloride-N,N-dimethylformamide adduct in DMF utilizing 40 grams of solution per gram of cotton. The reaction was run at 25°C for 1 hr. This solution was prepared by adding 7.2 parts of phosphorus trichloride to 92.8 parts of DMF. The resultant yarn was washed as in Example 2, and possessed 3.9% P, 0.2% N, and 0.5% Cl. It had a match test angle of 135°, quite acceptable for a flame resistant cotton textile.

We claim:

1. A process for preparing a fibrous crosslinked N,N-dimethylorthophosphorylchloridite ester of cellulose in textile form, which ester is characterized by its containing nitrogen, phosphorus, and chlorine in a 1:1:1 atomic ratio, said process comprising:
  - a. immersion of a fibrous cellulose textile in N,N-dimethylformamide at a temperature of about from 20°C to 30°C for a period of from 1 minute to 60 minutes to swell the fibers,
  - b. removal of excess N,N-dimethylformamide from the swollen cellulose,
  - c. immersion of the cellulosic textile in a solution containing about from 1% to 30% by weight of the 1:2 adduct of phosphorus trichloride with N,N-dimethylformamide, in a solvent containing 50%–100% N,N-dimethylformamide together with an inert aprotic diluent selected from the class consisting of chloroform, methylene chloride, carbon tetrachloride and perchloroethylene, at a temperature of from 20°C to 60°C for about from 1 minute to 180 minutes, in order to obtain reaction of the cellulose with the aforesaid adduct,
  - d. washing the cellulosic textile with N,N-dimethylformamide to remove unreacted adduct,
  - e. washing the cellulosic textile with a solvent selected from the group consisting of benzene and chloroform, to remove the N,N-dimethylformamide, and
  - f. drying the textile.
2. The process of claim 1 wherein the textile is in the form of a yarn.

3. The process of claim 1 wherein the textile is in the form of a fabric.

4. As a textile material, the fibrous crosslinked N,N-dimethylorthoformamoylphosphorochloridite ester of cellulose produced by the process of claim 1.

5. A process for preparing a fibrous, crosslinked, partially hydrolyzed N,N-dimethylorthoformamoylphosphite ester of cellulose in textile form, which ester is characterized by its nitrogen and phosphorus content, the absence of combined chlorine, and by its flame resistance and wrinkle resistance, said process comprising:

a. immersion of a fibrous cellulose textile in N,N-dimethylformamide at a temperature of about from 20°C to 30°C for a period of from 1 minute to 60 minutes to swell the fibers,

b. removal of excess N,N-dimethylformamide from the swollen cellulose,

c. immersion of the cellulosic textile in a solution containing about from 1% to 30% by weight of the 1:2 adduct of phosphorus trichloride with N,N-dimethylformamide, in a solvent containing 50%-100%, N,N-dimethylformamide together with

5

10

15

20

25

30

35

40

45

50

55

60

65

an inert aprotic diluent selected from the class consisting of chloroform, methylene chloride, carbon tetrachloride, and perchloroethylene, at a temperature of from 20°C to 60°C for about from 1 minute to 180 minutes, in order to obtain reaction of the cellulose with the aforesaid adduct,

d. washing the cellulosic textile with N,N-dimethylformamide to remove unreacted adduct,

e. washing the cellulosic textile with ice water and then washing at room temperature with water containing 0-10% acetic acid, to remove traces of reagents and solvents and combined chlorine, and

f. drying the textile.

6. The process of claim 5 wherein the textile is in the form of a yarn.

7. The process of claim 5 wherein the textile is in the form of a fabric.

8. As a textile material, the fibrous crosslinked partially hydrolyzed N,N-dimethylorthoformamoylphosphite ester of cellulose produced by the process of claim 5.

\* \* \* \* \*